



US007604049B2

(12) **United States Patent**  
**Vaidya et al.**

(10) **Patent No.:** **US 7,604,049 B2**  
(b4) **Date of Patent:** **Oct. 20, 2009**

(54) **POLYMERIC COMPOSITES, OILFIELD ELEMENTS COMPRISING SAME, AND METHODS OF USING SAME IN OILFIELD APPLICATIONS**

(75) Inventors: **Nitin Y. Vaidya**, Missouri City, TX (US); **Gregory H. Manke**, Overland Park, KS (US)

(73) Assignee: **Schlumberger Technology Corporation**, Sugar Land, TX (US)

(\*) Notice: Subject to any disclaimer, the term of this patent is extended or adjusted under 35 U.S.C. 154(b) by 258 days.

(21) Appl. No.: **11/306,119**

(22) Filed: **Dec. 16, 2005**

(65) **Prior Publication Data**

US 2007/0142547 A1 Jun. 21, 2007

(51) **Int. Cl.**  
**C08K 3/04** (2006.01)  
**E21B 41/00** (2006.01)

(52) **U.S. Cl.** ..... **166/244.1**; 166/105; 524/847; 977/902

(58) **Field of Classification Search** ..... 166/244.1, 166/105; 977/902; 428/402; 524/847  
See application file for complete search history.

(56) **References Cited**

U.S. PATENT DOCUMENTS

3,948,575 A \* 4/1976 Rosser ..... 175/325.2  
6,441,143 B1 8/2002 Koski  
6,555,945 B1 4/2003 Baughman et al.  
6,713,601 B2 3/2004 Phelps  
6,919,063 B2 \* 7/2005 Jang et al. ..... 423/445 B  
7,186,474 B2 \* 3/2007 Jang ..... 429/17  
7,373,991 B2 \* 5/2008 Vaidya et al. ..... 166/381  
2001/0016629 A1 8/2001 Mori et al.  
2002/0010248 A1 1/2002 Fomperie et al.  
2002/0054995 A1 5/2002 Mazurkiewicz

2002/0177650 A1 11/2002 Mori et al.  
2003/0036599 A1 2/2003 Mori et al.  
2004/0127621 A1 7/2004 Drzal et al.  
2005/0087343 A1 \* 4/2005 Du et al. ..... 166/369  
2005/0109502 A1 5/2005 Buc Slay et al.  
2005/0109544 A1 \* 5/2005 Ray et al. ..... 175/371  
2005/0112356 A1 \* 5/2005 Rynd et al. ..... 428/317.9  
2005/0161212 A1 7/2005 Leismer et al.  
2006/0219400 A1 10/2006 Xu et al.

(Continued)

FOREIGN PATENT DOCUMENTS

CA 2550161 A1 \* 6/2006

(Continued)

OTHER PUBLICATIONS

Messersmith, P.B. Giannelis, E.P., "Synthesis and Barrier Properties of Poly(eCaprolactone) Layered Silicate Nanocomposites", Journal of Polymer Science, Part A, Polymer Chemistry (33). 1995. 1047-1057.

(Continued)

Primary Examiner—Kenneth Thompson

(74) Attorney, Agent, or Firm—Osha Liang LLP; Kevin Brayton McGoff; James L. Kurka

(57)

ABSTRACT

Oilfield elements and assemblies are described comprising a polymeric matrix formed into an oilfield element, and a plurality of expanded graphitic nanoflakes and/or nanoplatelets dispersed in the polymeric matrix. Methods of using the oilfield elements and assemblies including same in oilfield operations are also described.

**19 Claims, 6 Drawing Sheets**



## U.S. PATENT DOCUMENTS

- 2007/0066491 A1\* 3/2007 Bicerano et al. .... 507/117  
 2007/0089877 A1 4/2007 Corre et al.  
 2007/0092432 A1\* 4/2007 Prud'Homme et al. .... 423/448  
 2007/0193736 A1 8/2007 Corre et al.

## FOREIGN PATENT DOCUMENTS

- |    |            |         |
|----|------------|---------|
| CN | 1869118 A  | 11/2006 |
| EP | 1533469 A1 | 5/2005  |
| RU | 2177092 C1 | 12/2001 |
| WO | 2004106420 | 12/2004 |
| WO | 2005009899 | 2/2005  |
| WO | 2005084172 | 9/2005  |

## OTHER PUBLICATIONS

- Neilson, L.E., "Models for the Permeability of Filled Polymer Systems." *J. Macromol. Sci. (Chem.)* A1(5). 1967. 929-942.  
 Okada, A., Kawasumi, M., Usuki, A., Kojima, Y., Kurauchi, T., and Kamigaito, O., "Nylon 6-Clay Hybrid." *Material Research Society Symposium Proceedings* (171). 1990. 45-50.  
 Pinnavaia, T. J., Beal, G.W., "Polymer-Clay Nanocomposites." John Wiley and Sons. Chichester. 2000. 207-211, 267-270.  
 Jing-Wei Shen, Xiao-Mei Chen, Wen-Yi Huang, Structure and Electrical Properties of Grafted Polypropylene/Graphite Nanocomposites Prepared by Solution Intercalation, *Journal of Applied Polymer Science*, 2003, pp. 1864-1869, vol. 88, Wiley Periodicals, Inc.  
 Wenge Zheng, Shing-Chung Wong, Hung-Jue Sue, Transport behavior of PMMA/expanded graphite nanocomposites, *Polymer* 73, 2002, pp. 6767-6773, Elsevier Science Ltd.  
 Charles Wilkie, *Nanocomposite Technology*, Back to Chemistry Department Website, 2001, Marquette University, U.S.  
 T.G. Gopakumar, D.J.Y.S. Page, Polypropylene/Graphite Nanocomposites by Thermo-Kinetic Mixing, *Polymer Engineering and Science*, Jun. 2004, pp. 1162-1169, vol. 44, No. 6, Wiley InterScience, Canada.  
 Guo-Hua Chen, Da-Jun Wu, Wen-Gui Weng, Wen-Li Yan, Dispersion of Graphite Nanosheets in a Polymer Matrix and the Conducting Property of the Nanocomposites, *Polymer Engineering and Science*, Dec. 2001, pp. 2148-2154, vol. 41, No. 12.  
 X.S. Du, M. Xiao, Y.Z. Meng, A.S. Hay, Facile synthesis of exfoliated and highly conductive poly(arylene disulfide)/graphite nanocomposites, *Polymers for Advanced Technologies*, 2004, pp. 320-323, vol. 15, John Wiley & Sons, Ltd.  
 X.S. Du, M. Xiao, Y.Z. Meng, Synthesis and Characterization of Polyaniline/Graphite Conducting Nanocomposites, *Journal of Polymer Science: Part B: Polymer Physics*, 2004, pp. 1972-1978, vol. 42, Wiley Periodicals, Inc.  
 Wengui Weng, Guohua Chen, Dajun Wu, Xiangfeng Chen, Jinrong Lu, Pingping Wang, Fabrication and Characterization of Nylon 6/Foliated Graphite Electrically Conducting Nanocomposite, *Journal of Polymer Science: Part B: Polymer Physics*, 2004, pp. 2844-2856, vol. 42, Wiley Periodicals, Inc.  
 Yu-Xun Pan, Zhong-Zhen Yu, Yu-Chun Ou, Guo-Hua Hu, A New Process of Fabricating Electrically Conducting Nylon 6/Graphite Nanocomposites via Intercalation Polymerization, *Journal of Polymer Science: Part B: Polymer Physics*, 2000, pp. 1626-1633, vol. 38, John Wiley & Sons, Inc.  
 Rui Zhang, Yuan Hu, Jiayan Xu, Weicheng Fan, Zuyao Chen, Qinan Wang, Preparation and Combustion Properties of Flame Retardant Styrene-Butyl Acrylate Copolymer/Graphite Oxide Nanocomposites, *Macromolecular Materials and Engineering*, 2004, pp. 355-359, vol. 289, Wiley-VCH Verlag GmbH & Co. KGaA, Weinheim, Germany.  
 Guohua Chen, Wengui Weng, Dajun Wu, Cuiling Wu, Nonlinear Conduction in Nylon-6/Foliated Graphite Nanocomposites above the Percolation Threshold, *Journal of Polymer Science: Part B: Polymer Physics*, 2004, pp. 155-167, vol. 42, Wiley Periodicals, Inc.  
 Guo-Hua Chen, Da-Jun Wu, Wen-Gui Weng, Wen-Li Yan, Preparation of Polymer/Graphite Conducting Nanocomposite by Intercalation Polymerization, *Journal of Applied Polymer Science*, 2001, pp. 2506-2513, vol. 82, John Wiley & Sons, Inc.  
 Wenge Zheng, Xuehong Lu, Shing-Chung Wong, Electrical and Mechanical Properties of Expanded Graphite-Reinforced High-Density Polyethylene, *Journal of Applied Polymer Science*, 2004, pp. 2781-2788, vol. 91, Wiley Periodicals, Inc.  
 Y. Kojima, K. Fukumori, A. Usuki, A. Okada, T. Kurauchi, Gas permeabilities in rubber-clay hybrid, *Journal of Materials Science Letters* 12, 1993, pp. 889-890, Chapman & Hall.  
 Yoshitsugu Kojima, Arimitsu Usuki, Masaya Kawasumi, Akane Okada, Yoshiaki Fukushima, Toshio Kurauchi, Osami Kamigaito, Mechanical properties of nylon 6-clay hybrid, *Journal of Materials Research*, 1996, p. 1185; vol. 8, No. 5, Materials Research Society.  
 Tie Lan, Padmananda D. Kaviratna, Thomas J. Pinnavaia, On the Nature of Polyimide-Clay Hybrid Composites, *Chem. Mater.* 1994, pp. 573-575, vol. 6, American Chemical Society.  
 K.E. Strawhecker, E Manias, Structure and Properties of Poly(vinyl alcohol)/Na<sup>+</sup> Montmorillonite Nanocomposites, *Chem. Mater.* 2000, pp. 2943-2949, vol. 12, American Chemical Society, U.S.  
 Ruijian Xu, Evangelos Manias, Alan J. Snyder, James Runt, New Biomedical Poly(urethane urea)-Layered Silicate Nanocomposites, *Macromolecules* 2001, pp. 337-339, vol. 34, American Chemical Society, U.S.

\* cited by examiner

**FIG. 1**

FIG. 2



**FIG. 3**

**FIG. 4A****FIG. 4B**

**FIG. 5A****FIG. 5B**

**FIG. 6A****FIG. 6B**

## 1

**POLYMERIC COMPOSITES, OILFIELD ELEMENTS COMPRISING SAME, AND METHODS OF USING SAME IN OILFIELD APPLICATIONS**

**BACKGROUND OF THE INVENTION**

**1. Field of Invention**

The present invention relates generally to the field of oilfield exploration, production, and testing, and more specifically to composites of polymeric materials and expanded graphite nanoflakes and/or nanoplatelets useful in such ventures.

**2. Related Art**

The polymeric materials that are used in oilfield services, and in particular downhole, require good resistance to diffusion/permeation of well fluids (gases and liquids). Unfilled polymers in general have low resistance to diffusion of chemicals that exist in wellbore environments and are more permeable to well fluids. In order to reduce the permeability of polymers, fillers such as carbon black, silica, talc, and the like are added to raw polymers. These fillers have a non-platy structure and/or have low anisotropy (aspect ratio) and therefore offer limited reduction in permeability of the resultant compound. Expanded/exfoliated graphite nanoflakes and nanoplatelets exist in platelet form, which can have aspect ratio exceeding 100, and preferably exceeding 200.

United States published patent application 20040127621, published Jul. 1, 2004, discloses methods of making high aspect ratio expanded graphite, and polymer composites made using crushed versions of the high aspect ratio expanded graphite. The reference reports the use of expanded graphite and its products such as nanoflakes and/or nanoplatelets as fillers in polymers. This reference provides methods of expanding/exfoliating graphite and information on surface treatment such as amine grafting, and acrylamide grafting. This reference also provides information on enhancement of mechanical properties and electrical conductivity of the resultant polymer compound. The reference claims the use of the polymeric composites for fuel cells, batteries and catalytic converters. A great number of polymer types are discussed, and the expanded graphite must have length less than 200 micrometers, or less than 200,000 nanometers, and thickness less than 0.1 micrometers, or less than 100 nanometers. While aspect ratio per se is not discussed, from the lengths and thicknesses disclosed, the aspect ratio may be 2000 or greater.

Nanocomposites are a relatively new class of composites that are particle-filled polymers for which at least one dimension of the dispersed particle is in the nanometer range ( $10^{-9}$  meter). Because of the size of the dispersed particles, certain nanocomposites may exhibit improved mechanical, thermal, optical, and electrical properties as compared to pure polymers or conventional composites. Many references disclose nanocomposites of various polymeric materials and graphite, and discuss one or more properties such as degree of crystallization, electrical and mechanical properties dispersion properties, combustion/flame retardant properties, and the like. Yet other references discuss similar properties of graphene-based composites, including barrier properties. Graphene is a sheet-like structure of hexagonal network of carbon atoms. A carbon nanotube comprises a graphene sheet rounded in a hollow form. Some references report applications of graphene-based composites for radiation and electromagnetic shielding, shrinkage and corrosion resistant coatings. Zheng et al., *J. Appl. Polym. Sci.*, 91:2781 (2004) and references 18-24 listed therein report the use of graphene

## 2

based polymers for barrier applications. So far as is known to the inventors herein, the use of graphite nanoflakes and/or nanoplatelets having aspect ratio exceeding 200, dispersed in a polymeric matrix or use as barrier materials has not been reported. The use of graphite nanoflakes and/or nanoplatelets in polymers, with the nanoflakes and/or nanoplatelets having aspect ratio exceeding 200 for use in oilfield applications has not been reported.

Many oilfield elements and tools utilize polymeric materials. For example, electrical submersible pumps (ESPs) are used for artificial lifting of fluid from a well or reservoir. An ESP typically comprises an electrical submersible motor, a seal section (sometimes referred to in the art as a protector) which functions to equalize the pressure between the inside of the system and the outside of the system and also acts as a reservoir for compensating the internal oil expansion from the motor; and a pump having one or more pump stages inside a housing. The protector may be formed of metal, as in a bellows device, or an elastomer, in which case the protector is sometimes referred to as a protector bag. Elastomers and other polymers may also be used in packer elements, blow out preventer elements, O-rings, gaskets, electrical insulators, pressure sealing elements for fluids, and in many other oilfield elements.

Common to all of these uses of polymers is exposure to hostile environments, such as hostile chemical and mechanical subterranean environments, that tend to unacceptably decrease the life and reliability of the polymers. There remains a need in the natural resources exploration, production, and testing field for improving reliability and life, as well as electrical properties in some instances, of polymeric components used in oilfield environments, such as protector bags, packer elements, pressure seals, valves, blow out preventer components, cable shielding and jacketing, and the like.

**SUMMARY OF THE INVENTION**

In accordance with the present invention, apparatus, oilfield elements comprising the apparatus, and methods of using the oilfield elements are described that reduce or overcome problems in previously known apparatus, oilfield elements, and methods. By combining the properties of polymers with the properties of expanded graphitic nanoflakes and/or nanoplatelets, the inventive apparatus, sometimes referred to herein as nanocomposites due to the size of the nanoflakes and/or nanoplatelets, may act together to increase the barrier, mechanical, and/or electrical properties of oilfield elements that comprise one or more apparatus of the invention. In particular, expanded graphitic nanoflakes and/or nanoplatelets may offer enhanced resistance to permeation of well fluids when incorporated into polymers. These platelets may provide resistance to diffusion and reduce the permeability of well fluids (gases and liquids) through the polymer nanocomposite. The use of expanded graphitic materials, particularly expanded graphite, offers a commercially feasible way to develop inexpensive polymer nanocomposites with good barrier and mechanical properties. Expanded graphite nanofillers are at least 500 times less expensive than carbon nanotubes and may offer comparable enhancements in mechanical properties at only a fractional cost of carbon nanotubes.

A first aspect of the invention is an apparatus comprising: a polymeric matrix formed into an oilfield element; a plurality of expanded graphitic nanoflakes and/or nanoplatelets dispersed (randomly or non-randomly) in the polymeric matrix.

As used herein the term "expanded graphitic" means a composition having a graphitic structure, more generally known as an  $sp^2$  structure formed from one or more elements along the second row of the Periodic Table of the Elements, such as boron, carbon, and nitrogen, that has had its layers separated by one or more thermal, chemical, and/or physical methods. Examples include expanded graphite, exfoliated graphite (which is known in the art as simply a form of expanded graphite), compositions based on boron and nitrogen, such as boron nitride (also known as hexagonal BN or "white graphite"), and the like. Boron nitrides have high thermal conductivity and are electrically insulating (dielectric constant ~4) as opposed to graphite, which is electrically conductive. Boron nitrides also exhibit low thermal expansion, are easily colorable, and chemically inert. Expanded graphite is an expanded graphitic within the invention comprising carbon in major proportion, derived from graphite, substituted graphite, or similar composition. The differing electrical conductivities of expanded graphite and expanded boron nitrides may offer a way to adjust the electrical conductivity of the polymeric matrix without changing the barrier properties significantly.

The term "nanoflake" has been introduced into the patent literature, such as in U.S. Pat. No. 6,916,434, in the context of what the inventors therein refer to as nanoflake carbon nanotubes. Nanoflake carbon nanotubes are defined therein as carbon tubes composed of a group of graphite sheets, which seem to be made up of a plurality of (usually many) flake-like graphite sheets formed into a patchwork or papier-mâché-like structure. As the inventors therein note, nanoflake carbon tubes are tubular carbon materials that are completely different in structure from single-walled carbon nanotubes in which a single graphite sheet is closed into a cylindrical form, or from concentric cylindrical or nested multi-walled carbon nanotubes in which a plurality of graphite sheets are each closed into a cylindrical form.

Similarly, the term "nanoplatelet" has been used in the patent literature, for example in U.S. Pat. No. 6,672,077 in the context of hydrogen storage. At least in this context, the inventors therein distinguished "nanoplatelets" from triangular lattice, nanofiber, single walled nanotube, multi walled nanotube, nanocage, nanococoon, nanorope, nanotorus, nanocoil, nanorod, nanowire, and fullerene structures. Nanoplatelets such as thin nanoplatelets, thick nanoplatelets, intercalated nanoplatelets, having thickness of about 0.3 nm to about 100 nm, and lateral size of about 5 nm to about 500 nm are described. While not being limited by these dimensions, which are given as useful examples herein only, these shapes and dimensions may be useful in the various aspects of the present invention.

In the present invention, the phrase "expanded graphitic nanoflakes and/or nanoplatelets" does not denote nanotubes, although it is not necessary that the expanded graphitic nanoflakes and/or nanoplatelets exclude curved contours; in other words, some or all of the expanded graphitic nanoflakes (or portions of each nanoflake) may have 3-dimensional shapes other than flat. As an example, expanded graphitic nanoflakes useful in the invention may be shaped as saddles, half-saddles, quarter-saddles, half-spheres, quarter spheres, cones, half-cones, bells, half-bells, horns, quarter-horns and the like, although the majority of each nanoflake, and the majority of nanoflakes as a whole may be flat.

Apparatus in accordance with the invention include those wherein the expanded graphitic nanoflakes and/or nanoplatelets have aspect ratio exceeding 100, and may exceed 200. The use of expanded and/or exfoliated graphitic nanoflakes and/or nanoplatelets with aspect ratio less than 200 are con-

sidered within the invention and may still enhance permeation resistance when compared with conventional nanoplatelet-like fillers such as clays, although the degree of enhancement may be lower. Apparatus of the invention 5 include those wherein the polymeric matrix includes both expanded graphitic platelets with aspect ratio less than 200 and exceeding 200, wherein the expanded nanoplatelets having aspect ratio less than 200 serve at least as a filler in the polymeric matrix for use in oilfield applications. The dimensions of the nanoflakes and/or nanoplatelets may vary greatly, but may be roughly hexagonal, circular, elliptical or rectangular. The aspect ratio and shapes which are most advantageously employed will depend on the desired end-use. Apparatus of the invention may be used in oilfield applications for 10 enhanced permeation resistance, and enhanced resistance to diffusion of gases and liquids at downhole conditions.

The various nanoflake and nanoplatelet structures useful in 15 the invention can assume heterogeneous forms. Heterogeneous forms include structures, where one part of the structure has a certain chemical composition, while another part of the structure has a different chemical composition. An example may be a nanoflake having two or more chemical 20 compositions or phases in different regions of the nanoflake. Heterogeneous forms may include different forms joined 25 together, for example where more than one of the above listed forms are joined into a larger irregular structure. For example, a "Frisbee", wherein a major portion is flat, but has a curved edge around the circumference. Moreover, all nanoflakes and 30 nanoplatelets may have cracks, dislocations, branches or other imperfections.

The polymeric matrix comprises one or more polymers 35 selected from natural and synthetic polymers, including those listed in ASTM D1600-92, "Standard Terminology for Abbreviated Terms Relating to Plastics", and ASTM D1418 for nitrile rubbers, blends of natural and synthetic polymers, and layered versions of polymers, wherein individual layers 40 may be the same or different in composition and thickness. The term "matrix" is not meant to exclude any particular form or morphology for the polymeric component and is used merely as a term of convenience in describing the apparatus of the invention. The term includes composite polymeric materials, such as, but not limited to, polymeric materials having 45 fillers, plasticizers, and fibers therein other than expanded graphitic nanoflakes and/or nanoplatelets. The polymeric matrix may comprise one or more thermoplastic polymers, such as polyolefins, polyamides, polyesters, thermoplastic polyurethanes and polyurea urethanes, copolymers, and blends thereof, and the like; one or more thermoset polymers, 50 such as phenolic resins, epoxy resins, and the like, and/or one or more elastomers (including natural and synthetic rubbers), and combinations thereof.

Apparatus of the invention include those wherein at least a 55 portion of the expanded graphitic nanoflakes and/or platelets are surface modified to enhanced permeation resistance when dispersed in the polymeric matrix. As a specific example, attaching functional groups on graphite nanoflakes and/or nanoplatelets may increase the bound rubber/polymer content 60 in the resultant polymeric matrix, which may enhance the permeation resistance of the resultant oilfield element. Functional groups that may enhance the bound polymer content will depend on the type of polymer or polymers comprising the polymeric matrix. For example, in polymers containing 65 nitrile groups, the introduction of carboxyl and/or hydroxyl groups may enhance the bound polymer content. Apparatus of the invention include those apparatus wherein the poly-

meric matrix comprises expanded graphitic nanoflakes and/or nanoplatelets having high aspect ratio and surface modification.

Apparatus within the invention include those wherein the oilfield element may be selected from packer elements, submersible pump motor protector bags, sensor protectors, blow out preventer elements, sucker rods, O-rings, T-rings, gaskets, pump shaft seals, tube seals, valve seals, seals and insulators used in electrical components, such as wire and cable semiconducting shielding and/or jacketing, which may inhibit the diffusion of gases such as methane, carbon dioxide, and hydrogen sulfide from well bore, through the cable and to the surface, power cable coverings, seals and bulkheads such as those used in fiber optic connections and other tools, and pressure sealing elements for fluids (gas, liquid, or combinations thereof). Apparatus of the invention include apparatus wherein the oilfield element is a submersible pump motor protector, which may or may not be integral with the motor, and may include integral instrumentation adapted to measure one or more downhole parameters.

Another aspect of the invention are oilfield assemblies for exploring for, testing for, or producing hydrocarbons, one oilfield assembly comprising:

- (a) one or more oilfield elements; and
- (b) one or more of the oilfield elements comprising a polymeric matrix having a plurality of expanded graphitic nanoflakes and/or nanoplatelets dispersed therein as described in the first aspect of the invention.

Yet another aspect of the invention are methods of exploring for, drilling for, or producing hydrocarbons, one method comprising:

- (a) selecting one or more oilfield elements having a component comprising a polymeric matrix having a plurality of expanded graphitic nanoflakes and/or nanoplatelets dispersed therein as described in the first aspect of the invention; and
- (b) using the oilfield element in an oilfield operation, thus exposing the oilfield element to an oilfield environment.

Methods of the invention may include, but are not limited to, running one or more oilfield elements into a wellbore using one or more surface oilfield elements, and/or retrieving the oilfield element from the wellbore. The oilfield environment during running and retrieving may be the same or different from the oilfield environment during use in the wellbore or at the surface.

Exposed surfaces of the polymeric matrix of the apparatus of the invention may optionally have a polymeric coating thereon, wherein the polymeric coating may be a condensed phase formed by any one or more processes. The coating may be conformal (i.e., the coating conforms to the surfaces of the polymeric matrix, which serves as a substrate for the coating), although this may not be necessary in all oilfield applications or all oilfield elements, or on all surfaces of the polymeric matrix. The coating may be formed from a vaporizable or depositable and polymerizable monomer, as well as particulate polymeric materials. The polymer in the coating may or may not be responsible for adhering the coating to the polymeric matrix, although the invention does not rule out adhesion aids, which are further discussed herein. A major portion of the polymeric coating may comprise a carbon or hetero-chain chain polymer. Useful carbon chain polymers may be selected from polytetrafluoroethylene, polychlorotrifluoroethylene, polycyclic aromatic hydrocarbons such as polynaphthalene, polyanthracene, and polyphenanthrene, and various polymeric coatings known generically as parylenes, such as Parylene N, Parylene C, Parylene D, and Parylene Nova HT.

Apparatus of the invention comprising one or more polymeric matrix polymers having expanded graphitic nanoflakes

and/or nanoplatelets dispersed therein should inhibit the diffusion and permeation of fluids when used in downhole and other oilfield service applications where one or more of the following conditions exist: 1) a differential pressure applied across polymeric component; 2) high temperature; 3) high pressure; 4) presence of low molecular weight molecules and gases such as methane, carbon dioxide, and hydrogen sulfide, and the like. Furthermore, the addition of exfoliated graphitic nanoflakes and/or nanoplatelets with either high aspect ratio (>200) or low aspect ratio may simultaneously enhance the electrical conductivity and barrier properties of the polymeric matrix, and therefore the oilfield elements. As a result, oilfield assemblies including semiconducting and permeability resistant shields in wire and cable applications, and in all other electrical and electronic components in oilfield applications, may be produced which have one or both of these requirements. Some examples include packaging of electronics such as sensors, multi-chip modules (MCM), and the like.

The various aspects of the invention will become more apparent upon review of the brief description of the drawings, the detailed description of the invention, and the claims that follow.

#### BRIEF DESCRIPTION OF THE DRAWINGS

The manner in which the objectives of the invention and other desirable characteristics can be obtained is explained in the following description and attached drawings in which:

FIG. 1 is a front elevation view of an exemplary electrical submersible pump disposed within a wellbore;

FIG. 2 is a diagrammatical cross-section of the pump of FIG. 1 having a polymeric matrix/nanoplatelet composite protector bag in accordance with the invention to separate well fluid from motor fluid, which is positively pressurized within the motor housing;

FIG. 3 is a schematic side elevation view, partially in cross-section, of a packer having polymeric matrix/nanoplatelet composite packer elements in accordance with the invention;

FIGS. 4A and 4B are schematic cross-sectional views of two reversing tools utilizing polymeric matrix/nanoplatelet composite components in accordance with the invention;

FIGS. 5A and 5B are schematic side elevation views of two bottom hole assemblies which may utilize polymeric matrix/nanoplatelet composite components in accordance with the invention; and

FIGS. 6A and 6B are schematic cross-sectional views of a flow control valve that may be utilized to control the flow of petroleum production or well fluids out of specific zones in a well or reservoir, or injection of fluid into specific zones, the valve utilizing polymeric matrix/nanoplatelet composite components in accordance with the invention.

It is to be noted, however, that the appended drawings are not to scale and illustrate only typical embodiments of this invention, and are therefore not to be considered limiting of its scope, for the invention may admit to other equally effective embodiments.

#### DETAILED DESCRIPTION

In the following description, numerous details are set forth to provide an understanding of the present invention. However, it will be understood by those skilled in the art that the present invention may be practiced without these details and that numerous variations or modifications from the described embodiments may be possible.

All phrases, derivations, collocations and multiword expressions used herein, in particular in the claims that fol-

low, are expressly not limited to nouns and verbs. It is apparent that meanings are not just expressed by nouns and verbs or single words. Languages use a variety of ways to express content. The existence of inventive concepts and the ways in which these are expressed varies in language-cultures. For example, many lexicalized compounds in Germanic languages are often expressed as adjective-noun combinations, noun-preposition-noun combinations or derivations in Romanic languages. The possibility to include phrases, derivations and collocations in the claims is essential for high-quality patents, making it possible to reduce expressions to their conceptual content, and all possible conceptual combinations of words that are compatible with such content (either within a language or across languages) are intended to be included in the used phrases.

The invention describes polymeric matrix/nanoplatelet and/or nanoflake composite components useful in oilfield applications, including exploration, drilling, testing, completion, and production activities. As used herein the term "oil-field" includes land based (surface and sub-surface) and sub-seabed applications, and in certain instances seawater applications, such as when exploration, drilling, or production equipment is deployed through seawater. The term "oil-field" as used herein includes oil and gas reservoirs, and formations or portions of formations where oil and gas are expected but may ultimately only contain water, brine, or some other composition. A typical use of the polymeric matrix/nanoplatelet composite components will be in down-hole applications, such as pumping fluids from or into well-bores, although the invention is not so limited.

#### Expanded Graphitic Nanoflakes and Nanoplatelets

It is well known in rubber industry that the use of fillers may reduce the swelling and permeability of polymeric materials. In general, the reduction in swelling and permeability increases as the filler concentration is increased. The permeability of polymeric materials may also depend on the shape and aspect ratio of the filler particles. Platelet like fillers such as nanoclays, preferably with small thickness (<0.1 micrometer) and length less than 200 micrometers, when aligned, may create a tortuous path for diffusing fluid molecules and therefore may enhance the barrier properties of the resultant materials compared with barrier properties of raw polymer of the same composition and morphology. When individual nanoparticles are dispersed in such a way that the particles separate into very thin individual platelets or layers, with high aspect ratio (>200 approximately), this process is called exfoliation. Exfoliation of conventional clay-based fillers is difficult and may occur while mixing the clay filler into the polymer.

In the case of graphitic nanoflakes and/or nanoplatelets useful in the present invention, the particles may be surface treated and expanded/exfoliated by application of heat either before or after it is mixed with the polymer or polymers forming the polymeric matrix. The use of expanded graphitic nanoflakes and/or nanoplatelets enables easier mixing and exfoliation of the nanoflakes and/or nanoplatelets into a given polymer as compared to nanoclay fillers. This provides a commercially feasible method involving melt or mechanical mixing of the polymer with the expanded graphitic nanoplatelets without the use of solvents, or with very little solvent.

Suitable graphitic nanoflakes and nanoplatelets under proper conditions are defined herein as materials comprised primarily of two elements having at least one dimension in the nanometer-size. A nanometer (nm) is  $10^{-9}$  meter, therefore, nanometer-size range encompasses from about 1 to 999

nm. Graphitic nanoflakes and nanoplatelets useful in the invention may be natural, modified, or synthetic in nature, or any combination thereof.

The expanded graphitic nanoflakes and/or platelets useful in the invention may be prepared by expanding expandable graphitic materials from about 40:1 to about 300:1 expansion ratio. With a volume expansion ratio of less than 40:1, sufficient dispersal of the nanoplatelet and/or nanoflakes may not be obtained, while if expanded over 300:1, the desired structure (if any) of the graphitic nanoflakes and/or nanoplatelets may be destroyed. The particle size may range from about 44 to about 300 micron before blending into the polymer or polymers that will make up the polymeric matrix. The particle size (length) may change during the process of blending with polymer/elastomer. The thickness of individual platelets may range from about 10 nm to about 50 nm in the polymeric matrix.

#### Polymeric Matrix Materials

Polymeric matrix materials useful in the invention may be selected from natural and synthetic polymers, blends of natural and synthetic polymers, and layered versions of polymers, wherein individual layers may be the same or different in composition and thickness. The term "polymeric matrix" includes composite polymeric materials, such as, but not limited to, polymeric materials having "non-nanometer scale" fillers, plasticizers, and fibers therein, wherein "non-nanometer-scale" refers to 1000 nm (1 micrometer) or larger. The polymeric matrix may comprise one or more thermoplastic polymers, one or more thermoset and/or thermally cured polymers, one or more elastomers, composite materials, and combinations thereof.

One class of useful polymeric matrix materials are the elastomers. "Elastomer" as used herein is a generic term for substances emulating natural rubber in that they stretch under tension, have a high tensile strength, retract rapidly, and substantially recover their original dimensions. The term includes natural and man-made elastomers, and the elastomer may be a thermoplastic elastomer or a non-thermoplastic elastomer. The term includes blends (physical mixtures) of elastomers, as well as copolymers, terpolymers, and multi-polymers. Examples include ethylene-propylene-diene polymer (EPDM), various nitrile rubbers which are copolymers of butadiene and acrylonitrile such as Buna-N (also known as standard nitrile and NBR). By varying the acrylonitrile content, elastomers with improved oil/fuel swell or with improved low-temperature performance can be achieved. Specialty versions of carboxylated high-acrylonitrile butadiene copolymers (XNBR) provide improved abrasion resistance, and hydrogenated versions of these copolymers (HNBR) provide improved chemical and ozone resistance elastomers. Carboxylated HNBR is also known. Other useful rubbers include polyvinylchloride-nitrile butadiene (PVC-NBR) blends, chlorinated polyethylene (CM), chlorinated sulfonate polyethylene (CSM), aliphatic polyesters with chlorinated side chains such as epichlorohydrin homopolymer (CO), epichlorohydrin copolymer (ECO), and epichlorohydrin terpolymer (GECO), polyacrylate rubbers such as ethylene-acrylate copolymer (ACM), ethylene-acrylate terpolymers (AEM), EPR, elastomers of ethylene and propylene, sometimes with a third monomer, such as ethylene-propylene copolymer (EPM), ethylene vinyl acetate copolymers (EVM), fluorocarbon polymers (FKM), copolymers of poly(vinylidene fluoride) and hexafluoropropylene (VF2/HFP), terpolymers of poly(vinylidene fluoride), hexafluoropropylene, and tetrafluoroethylene (VF2/HFP/TFE), terpolymers of poly(vinylidene fluoride), polyvinyl

methyl ether and tetrafluoroethylene (VF<sub>2</sub>/PVME/TFE), terpolymers of poly(vinylidene fluoride), hexafluoropropylene, and tetrafluoroethylene (VF<sub>2</sub>/HPF/TFE), terpolymers of poly(vinylidene fluoride), tetrafluoroethylene, and propylene (VF<sub>2</sub>/TFE/P), perfluoroelastomers such as tetrafluoroethylene perfluoroelastomers (FFKM), highly fluorinated elastomers (FEPM), butadiene rubber (BR), polychloroprene rubber (CR), polyisoprene rubber (IR), . . . (IM), polynorbornenes, polysulfide rubbers (OT and EOT), polyurethanes (AU) and (EU), silicone rubbers (MQ), vinyl silicone rubbers (VMQ), fluoromethyl silicone rubber (FMQ), fluorovinyl silicone rubbers (FVMQ), phenylmethyl silicone rubbers (PMQ), styrene-butadiene rubbers (SBR), copolymers of isobutylene and isoprene known as butyl rubbers (IIR), brominated copolymers of isobutylene and isoprene (BIIR) and chlorinated copolymers of isobutylene and isoprene (CIIR).

Suitable examples of useable fluoroelastomers are copolymers of vinylidene fluoride and hexafluoropropylene and terpolymers of vinylidene fluoride, hexafluoropropylene and tetrafluoroethylene. The fluoroelastomers suitable for use in the disclosed invention are elastomers that comprise one or more vinylidene fluoride units (VF<sub>2</sub> or VdF), one or more hexafluoropropylene units (HFP), one or more tetrafluoroethylene units (TFE), one or more chlorotrifluoroethylene (CTFE) units, and/or one or more perfluoro(alkyl vinyl ether) units (PAVE) such as perfluoro(methyl vinyl ether)(PMVE), perfluoro(ethyl vinyl ether)(PEVE), and perfluoro(propyl vinyl ether)(PPVE). These elastomers can be homopolymers or copolymers. Particularly suitable are fluoroelastomers containing vinylidene fluoride units, hexafluoropropylene units, and, optionally, tetrafluoroethylene units and fluoroelastomers containing vinylidene fluoride units, perfluoroalkyl perfluorovinyl ether units, and tetrafluoroethylene units, such as the vinylidene fluoride type fluoroelastomer known under the trade designation Aflas®, available from Asahi Glass Co., Ltd. Especially suitable are copolymers of vinylidene fluoride and hexafluoropropylene units. If the fluoropolymers contain vinylidene fluoride units, preferably the polymers contain up to 40 mole % VF<sub>2</sub> units, e.g., 30-40 mole %. If the fluoropolymers contain hexafluoropropylene units, preferably the polymers contain up to 70 mole % HFP units. If the fluoropolymers contain tetrafluoroethylene units, preferably the polymers contain up to 10 mole % TFE units. When the fluoropolymers contain chlorotrifluoroethylene preferably the polymers contain up to 10 mole % CTFE units. When the fluoropolymers contain perfluoro(methyl vinyl ether) units, preferably the polymers contain up to 5 mole % PMVE units. When the fluoropolymers contain perfluoro(ethyl vinyl ether) units, preferably the polymers contain up to 5 mole % PEVE units. When the fluoropolymers contain perfluoro(propyl vinyl ether) units, preferably the polymers contain up to 5 mole % PPVE units. The fluoropolymers preferably contain 66%-70% fluorine. One suitable commercially available fluoroelastomer is that known under the trade designation Technoflon FOR HS® sold by Ausimont USA. This material contains Bisphenol AF, manufactured by Halocarbon Products Corp. Another commercially available fluoroelastomer is known under the trade designation Viton® AL 200, by DuPont Dow, which is a terpolymer of VF<sub>2</sub>, HFP, and TFE monomers containing 67% fluorine. Another suitable commercially available fluoroelastomer is Viton® AL 300, by DuPont Dow. A blend of the terpolymers known under the trade designations Viton® AL 300 and Viton® AL 600 can also be used (e.g., one-third AL-600 and two-thirds AL-300). Other useful elastomers include products known under the trade designations 7182B and 7182D from Seals Eastern, Red Bank, N.J.; the product known under the trade designation

FL80-4 available from Oil States Industries, Inc., Arlington, Tex.; and the product known under the trade designation DMS005 available from Duromould, Ltd., Londonderry, Northern Ireland.

5 Thermoplastic elastomers are generally the reaction product of a low equivalent molecular weight polyfunctional monomer and a high equivalent molecular weight polyfunctional monomer, wherein the low equivalent weight polyfunctional monomer is capable, on polymerization, of forming 10 a hard segment (and, in conjunction with other hard segments, crystalline hard regions or domains) and the high equivalent weight polyfunctional monomer is capable, on polymerization, of producing soft, flexible chains connecting the hard regions or domains.

15 "Thermoplastic elastomers" differ from "thermoplastics" and "elastomers" in that thermoplastic elastomers, upon heating above the melting temperature of the hard regions, form a 20 homogeneous melt which can be processed by thermoplastic techniques (unlike elastomers), such as injection molding, extrusion, blow molding, and the like. Subsequent cooling leads again to segregation of hard and soft regions resulting in a material having elastomeric properties, however, which 25 does not occur with thermoplastics. Commercially available thermoplastic elastomers include segmented polyester thermoplastic elastomers, segmented polyurethane thermoplastic elastomers, segmented polyamide thermoplastic elastomers, blends of thermoplastic elastomers and thermoplastic polymers, and ionomeric thermoplastic elastomers.

30 "Segmented thermoplastic elastomer", as used herein, refers to the sub-class of thermoplastic elastomers which are based on polymers which are the reaction product of a high equivalent weight polyfunctional monomer and a low equivalent weight polyfunctional monomer.

35 "Ionomeric thermoplastic elastomers" refers to a sub-class of thermoplastic elastomers based on ionic polymers (ionomers). Ionomeric thermoplastic elastomers are composed of two or more flexible polymeric chains bound together at a plurality of positions by ionic associations or clusters. The ionomers are typically prepared by copolymerization of a 40 functionalized monomer with an olefinic unsaturated monomer, or direct functionalization of a preformed polymer. Carboxyl-functionalized ionomers are obtained by direct copolymerization of acrylic or methacrylic acid with ethylene, styrene and similar comonomers by free-radical copolymerization. 45 The resulting copolymer is generally available as the free acid, which can be neutralized to the degree desired with metal hydroxides, metal acetates, and similar salts.

50 Another useful class of polymeric matrix materials are thermoplastic materials. A thermoplastic material is defined as a polymeric material (preferably, an organic polymeric material) that softens and melts when exposed to elevated temperatures and generally returns to its original condition, i.e., its original physical state, when cooled to ambient temperatures. During the manufacturing process of an oilfield 55 element, the thermoplastic material may be heated above its softening temperature, and preferably above its melting temperature, to cause it to flow and form the desired shape of the oilfield element. After the desired shape is formed, the thermoplastic substrate is cooled and solidified. In this way, thermoplastic materials (including thermoplastic elastomers) can be molded into various shapes and sizes.

56 Moldable thermoplastic materials that may be used are those having a high melting temperature, good heat resistant properties, and good toughness properties such that the oilfield element or assemblies containing these materials operably 60 withstand oilfield conditions without substantially deforming or disintegrating.

## 11

Thermoplastic polymers useful as polymeric matrix materials are those able to withstand expected temperatures, temperature changes, and temperature differentials (for example a temperature differential from one surface of a gasket to the other surface material to the other surface) during use, as well as expected pressures, pressure changes, and pressure differentials during use, with a safety margin on temperature and pressure appropriate for each application.

Examples of thermoplastic materials suitable as polymeric matrix materials in oilfield elements according to the present invention include polyolefins, polyamides, polyesters, thermoplastic polyurethanes and polyurea urethanes, PP, PE, PP-PE copolymer, PVC and other polyolefins, polyamides, polyetheretherketones (PEEK), polyaryletherketones (PAEK), polyetherimides (PEI), copolymers of tetrafluoroethylene and perfluorovinylether (PFA), perfluoroalkoxy copolymers (MFA), polycarbonates, polyetherimides, polyesters, polysulfones, polystyrenes, acrylonitrile-butadiene-styrene block copolymers, acetal polymers, polyamides, copolymers, blends, and other combinations thereof, and the like. Of this list, polyamides and polyesters may provide better performance. Polyamide materials are useful at least because they are inherently tough and heat resistant, typically provide good adhesion to coatings without priming, and are relatively inexpensive. Polyamide resin materials may be characterized by having an amide group, i.e.,  $-\text{C}(\text{O})\text{NH}-$ . Various types of polyamide resin materials, i.e., nylons, can be used, such as nylon 6/6 or nylon 6. Of these, nylon 6 may be used if a phenolic-based coating is used because of the excellent adhesion between nylon 6 and phenolic-based coatings. Nylon 6/6 is a condensation product of adipic acid and hexamethylene-diamine. Nylon 6/6 has a melting point of about 264° C. and a tensile strength of about 770 kg/cm<sup>2</sup>. Nylon 6 is a polymer of  $\epsilon$ -caprolactam. Nylon 6 has a melting point of about 223° C. and a tensile strength of about 700 kg/cm<sup>2</sup>. Examples of commercially available nylon resins useable as substrates in oilfield elements according to the present invention include those known under the trade designations "Vydyn" from Solutia, St. Louis, Mo.; "Zytel" and "Minion" both from DuPont, Wilmington, Del.; "Trogamid T" from Degussa Corporation, Parsippany, N.J.; "Capron" from BASF, Florham Park, N.J.; "Nydur" from Mobay, Inc., Pittsburgh, Pa.; and "Ultramid" from BASF Corp., Parsippany, N.J. Mineral-filled thermoplastic materials can be used, such as the mineral-filled nylon 6 resin "Minion", from DuPont.

Suitable thermoset (thermally cured) polymers for use as polymeric matrices in the present invention include phenolic resins, epoxy resins, phenoxy, phenolic, ester, polyurethane, polyurea, and the like, and include those discussed in relation to polymeric coatings, which discussion follows, although the precursor solutions need not be coatable, and may therefore omit certain ingredients, such as diluents. Thermoset molding compositions known in the art are generally thermosetting resins containing inorganic fillers and/or fibers. Upon heating, thermoset monomers initially exhibit viscosities low enough to allow for melt processing and molding of an article from the filled monomer composition. Upon further heating, the thermosetting monomers react and cure to form hard resins with high stiffness. Thermoset polymeric substrates useful in the invention may be manufactured by any method known in the art. These methods include, but are not limited to, reaction injection molding, resin transfer molding, and other processes wherein dry fiber reinforcement plies (preforms) are loaded in a mold cavity whose surfaces define the ultimate configuration of the article to be fabricated, whereupon a flowable resin is injected, or vacuumed, under pressure into the mold cavity (mold plenum) thereby to produce

## 12

the article, or to saturate/wet the fiber reinforcement preforms, where provided. After the resinated preforms are cured in the mold plenum, the finished article is removed from the mold. As one non-limiting example of a useable thermosettable polymer precursor composition, U.S. Pat. No. 6,878,782 discloses a curable composition including a functionalized poly(arylene ether); an alkenyl aromatic monomer; an acryloyl monomer; and a polymeric additive having a glass transition temperature less than or equal to 100° C., and a 10 Young's modulus less than or equal to 1000 megapascals at 25° C. The polymeric additive is soluble in the combined functionalized poly(arylene ether), alkenyl aromatic monomer, and acryloyl monomer at a temperature less than or equal to 50° C. The composition exhibits low shrinkage on curing and improved surface smoothness. It is useful, for example, in the manufacture of sucker rods.

## Adhesion Promoters, Coupling Agents and other Optional Ingredients

The polymeric matrix may comprise other ingredients in addition to the expanded graphitic nanoflakes and/or nanoplatelets, such as fillers, coupling agents, suspension agents, pigments, and the like.

For embodiments wherein a better bond between the polymeric matrix and any protective coating therefore is desired, mechanical and/or chemical adhesion promotion (priming) techniques may be used. For example, if the polymeric matrix is a thermoplastic polycarbonate, polyetherimide, polyester, polysulfone, or polystyrene material, use of a primer may be preferred to enhance the adhesion between the matrix and a coating. The term "primer" as used in this context is meant to include both mechanical and chemical type primers or priming processes. Examples of mechanical priming processes include, but are not limited to, corona treatment and scuffing, both of which increase the surface area of the polymeric matrix. An example of a preferred chemical primer is a colloidal dispersion of, for example, polyurethane, acetone, isopropanol, water, and a colloidal oxide of silicon, as taught by U.S. Pat. No. 4,906,523, which is incorporated herein by reference.

Besides the polymeric material, the polymeric matrix may include an effective amount of a fibrous reinforcing material. Herein, an "effective amount" of a fibrous reinforcing material is a sufficient amount to impart at least improvement in the physical characteristics of the oilfield element, i.e., heat resistance, toughness, flexibility, stiffness, shape control, adhesion, etc., but not so much fibrous reinforcing material as to give rise to any significant number of voids and detrimentally affect the structural integrity of the oilfield element. The amount of the fibrous reinforcing material in the polymeric matrix may be any amount that does not substantially detrimentally affect the desired barrier properties achieved by the graphitic nanoflakes and/or nanoplatelets, and may be within a range of about 1-40 parts, or within a range of about 5-35 parts, or within a range of about 15-30 parts by weight, for every 100 parts by weight of polymer.

The fibrous reinforcing material may be in the form of individual fibers or fibrous strands, or in the form of a fiber mat or web. The mat or web can be either in a woven or nonwoven matrix form. Examples of useful reinforcing fibers in applications of the present invention include metallic fibers or nonmetallic fibers. The nonmetallic fibers include glass fibers, carbon fibers, mineral fibers, synthetic or natural fibers formed of heat resistant organic materials, or fibers made from ceramic materials.

By "heat resistant" organic fibers, it is meant that useable organic fibers must be resistant to melting, or otherwise

breaking down, under the conditions of manufacture and use of the oilfield elements of the present invention. Examples of useful natural organic fibers include wool, silk, cotton, or cellulose. Examples of useful synthetic organic fibers include polyvinyl alcohol fibers, polyester fibers, rayon fibers, polyamide fibers, acrylic fibers, aramid fibers, or phenolic fibers. Generally, any ceramic fiber is useful in applications of the present invention. An example of a ceramic fiber suitable for the present invention is "Nextel" which is commercially available from 3M Co., St. Paul, Minn. Glass fibers may be used, at least because they impart desirable characteristics to the oilfield elements and are relatively inexpensive. Furthermore, suitable interfacial binding agents exist to enhance adhesion of glass fibers to thermoplastic materials. Glass fibers are typically classified using a letter grade. For example, E glass (for electrical) and S glass (for strength). Letter codes also designate diameter ranges, for example, size "D" represents a filament of diameter of about 6 micrometers and size "G" represents a filament of diameter of about 10 micrometers. Useful grades of glass fibers include both E glass and S glass of filament designations D through U. Preferred grades of glass fibers include E glass of filament designation "G" and S glass of filament designation "G." Commercially available glass fibers are available from Specialty Glass Inc., Oldsmar, Fla.; Johns Manville, Littleton, Colo.; and Mo-Sci Corporation, Rolla, Mo. If glass fibers are used, the glass fibers may be accompanied by an interfacial binding agent, i.e., a coupling agent, such as a silane coupling agent, to improve the adhesion to the thermoplastic material. Examples of silane coupling agents include "Z-6020" and "Z-6040," available from Dow Corning Corp., Midland, Mich.

The polymer nanocomposites of the present invention may further include an effective amount of a toughening agent. This will be preferred for certain applications. A primary purpose of the toughening agent is to increase the impact strength of the oilfield elements. By "an effective amount of a toughening agent" it is meant that the toughening agent is present in an amount to impart at least improvement in the polymeric matrix toughness without it becoming too flexible. Polymeric matrices of the present invention preferably include sufficient toughening agent to achieve the desirable impact test values listed above. An oilfield element polymeric matrix of the present invention may contain between about 1 part and about 30 parts of the toughening agent, based upon 100 parts by weight of the polymeric matrix. For example, the less elastomeric characteristics a toughening agent possesses, the larger quantity of the toughening agent may be required to impart desirable properties to the oilfield elements of the present invention. Toughening agents that impart desirable stiffness characteristics to the oilfield elements of the present invention include rubber-type polymers and plasticizers. Of these, the rubber toughening agents may be mentioned, and synthetic elastomers. Examples of preferred toughening agents, i.e., rubber tougheners and plasticizers, include: toluenesulfonamide derivatives (such as a mixture of N-butyl- and N-ethyl-p-toluenesulfonamide, commercially available from Akzo Chemicals, Chicago, Ill., under the trade designation "Ketjenflex 8"); styrene butadiene copolymers; poly-ether backbone polyamides (commercially available from Atochem, Glen Rock, N.J., under the trade designation "Pebax"); rubber-polyamide copolymers (commercially available from DuPont, Wilmington, Del., under the trade designation "Zytel FN"); and functionalized triblock polymers of styrene-(ethylene butylene)-styrene (commercially available from Shell Chemical Co., Houston, Tex., under the trade designation "Kraton FG1901"); and mixtures of these

materials. Of this group, rubber-polyamide copolymers and styrene-(ethylene butylene)-styrene triblock polymers may be used, at least because of the beneficial characteristics they may impart. Commercial compositions of toughener and thermoplastic material are available, for example, under the designation "Ultramid" from BASF Corp., Parsippany, N.J. Specifically, "Ultramid B3ZG6" is a nylon resin containing a toughening agent and glass fibers that is useful in the present invention.

Other such materials that may be added to the polymeric matrix for certain applications of the present invention include inorganic or organic fillers. Inorganic fillers are also known as mineral fillers. A filler is defined as a particulate material, typically having a particle size less than about 100 micrometers, preferably less than about 50 micrometers, but larger than about 1 micrometer. Examples of useful fillers for applications of the present invention include carbon black, calcium carbonate, silica, calcium metasilicate, cryolite, phenolic fillers, or polyvinyl alcohol fillers. If a filler is used, it is theorized that the filler may fill in between the nanoflakes and/or nanoplatelets, or between reinforcing fibers if used, and may prevent crack propagation through the substrate. Typically, a filler would not be used in an amount greater than about 20%, based on the weight of the polymeric matrix.

Other useful materials or components that may be added to the polymeric matrix for certain applications of the present invention include, but are not limited to, oils, antistatic agents, flame retardants, heat stabilizers, ultraviolet stabilizers, internal lubricants, antioxidants, and processing aids. One would not typically use more of these components than needed for desired results.

The apparatus of the invention, in particular the polymeric matrix, if filled with fillers, may also contain coupling agents. When an organic polymeric matrix has an inorganic filler, a coupling agent may be desired. Coupling agents may operate through two different reactive functionalities: an organofunctional moiety and an inorganic functional moiety. When a resin/filler mixture is modified with a coupling agent, the organofunctional group of the coupling agent becomes bonded to or otherwise attracted to or associated with the uncured resin. The inorganic functional moiety appears to generate a similar association with the dispersed inorganic filler. Thus, the coupling agent acts as a bridge between the organic resin and the inorganic filler at the resin/filler interface. In various systems this results in:

1. Reduced viscosity of the resin/filler dispersion. Such a dispersion, during a process of preparing a coated substrate, generally facilitates application.

2. Enhanced suspendability of the filler in the resin, i.e., decreasing the likelihood that suspended or dispersed filler will settle out from the resin/filler suspension during storing or processing to manufacture oilfield elements.

3. Improved product performance due to enhanced operation lifetime, for example through increased water resistance or general overall observed increase in strength and integrity of the bonding system.

Herein, the term "coupling agent" includes mixtures of coupling agents. An example of a coupling agent that may be found suitable for this invention is gamma-methacryloxypropyltrimethoxy silane known under the trade designation "Silquest A-174" from GE Silicones, Wilton, Conn. Other suitable coupling agents are zircoaluminates, and titanates.

#### Coatings

"Coating" as used herein as a noun, means a condensed phase formed by any one or more processes. The coating may be conformal (i.e., the coating conforms to the surfaces of the

polymeric matrix), although this may not be necessary in all oilfield applications or all oilfield elements, or on all surfaces of the polymeric matrix. Conformal coatings based on urethane, acrylic, silicone, and epoxy chemistries are known, primarily in the electronics and computer industries (printed circuit boards, for example). Another useful conformal coating includes those formed by vaporization or sublimation of, and subsequent pyrolyzation and condensation of monomers or dimers and polymerized to form a continuous polymer film, such as the class of polymeric coatings based on poly (p-xylylene), commonly known as Parylene. For example, Parylene N coatings may be formed by vaporization or sublimation of a dimer, and subsequent pyrolyzation and condensation of the divalent radicals to form the parylene polymer, although the vaporization is not strictly necessary.

Another class of useful polymeric coatings are thermally curable coatings derived from coatable, thermally curable coating precursor solutions, such as those described in U.S. Pat. No. 5,178,646, incorporated by reference herein. Coatable, thermally curable coating precursor solutions may comprise a 30-95% solids solution, or 60-80% solids solution of a thermally curable resin having a plurality of pendant methylol groups, the balance of the solution comprising water and a reactive diluent. The term "coatable", as used herein, means that the solutions of the invention may be coated or sprayed onto polymeric substrates using coating devices which are conventional in the spray coating art, such as knife coaters, roll coaters, flow-bar coaters, electrospray coaters, ultrasonic coaters, gas-atomizing spray coaters, and the like. The term "percent solids" means the weight percent organic material that would remain upon application of curing conditions. Percent solids below about 30% are not practical to use because of VOC emissions, while above about 95% solids the resin solutions are difficult to render coatable, even when heated.

The term "diluent" is used in the sense that the reactive diluent dilutes the concentration of thermally curable resin in the solution, and does not mean that the solutions necessarily decrease in viscosity. The thermally curable resin may be the reaction product of a non-aldehyde and an aldehyde, the non-aldehyde selected from ureas and phenolics. The reactive diluent has at least one functional group which is independently reactive with the pendant methylol groups and with the aldehyde.

Optionally, useful coatable, thermally curable polymeric coating precursor solutions may include up to about 50 weight percent (of the total weight of thermally curable resin) of ethylenically unsaturated monomers. These monomers, such as tri- and tetra-ethylene glycol diacrylate, are radiation curable and can reduce the overall cure time of the thermally curable resins by providing a mechanism for pre-cure gelation of the thermally curable resin.

Two other classes of useful coatings are condensation curable and addition polymerizable resins, wherein the addition polymerizable resins are derived from a polymer precursor which polymerizes upon exposure to a non-thermal energy source which aids in the initiation of the polymerization or curing process. Examples of non-thermal energy sources include electron beam, ultraviolet light, visible light, and other non-thermal radiation. During this polymerization process, the resin is polymerized and the polymer precursor is converted into a solidified polymeric coating. Upon solidification of the polymer precursor, the coating is formed. The polymer in the coating is also generally responsible for adhering the coating to the polymeric substrate, however the invention is not so limited. Addition polymerizable resins are readily cured by exposure to radiation energy. Addition poly-

merizable resins can polymerize through a cationic mechanism or a free radical mechanism. Depending upon the energy source that is utilized and the polymer precursor chemistry, a curing agent, initiator, or catalyst may be used to help initiate the polymerization.

Examples of useful organic resins to form these classes of polymeric coating include the before-mentioned methylol-containing resins such as phenolic resins, urea-formaldehyde resins, and melamine formaldehyde resins; acrylated urethanes; acrylated epoxies; ethylenically unsaturated compounds; aminoplast derivatives having pendant unsaturated carbonyl groups; isocyanurate derivatives having at least one pendant acrylate group; isocyanate derivatives having at least one pendant acrylate group; vinyl ethers; epoxy resins; and mixtures and combinations thereof. The term "acrylate" encompasses acrylates and methacrylates.

Phenolic resins are widely used in industry because of their thermal properties, availability, and cost. Both types of phenolic resins, resole and novolac, are useful in the invention.

Examples of commercially available phenolic resins include those known by the tradenames "Durez" and "Varcum" from Durez Corporation, a subsidiary of Sumitomo Bakelite Co., Ltd.; "Resinox" from Monsanto; "Aerofene" from Ashland Chemical Co. and "Aerotap" from Ashland Chemical Co.

Acrylated urethanes are diacrylate esters of hydroxy-terminated, isocyanate (NCO) extended polyesters or polyethers. Examples of commercially available acrylated urethanes include those known under the trade designations "UVITHANE 782", available from Morton Thiokol Chemical, and "CMD 6600", "CMD 8400", and "CMD 8805", available from Radcure Specialties.

Acrylated epoxies are diacrylate esters of epoxy resins, such as the diacrylate esters of Bisphenol A epoxy resin. Examples of commercially available acrylated epoxies include those known under the trade designations "CMD 3500", "CMD 3600", and "CMD 3700", available from Radcure Specialties.

Ethylenically unsaturated resins include both monomeric and polymeric compounds that contain atoms of carbon, hydrogen, and oxygen, and optionally, nitrogen and the halogens. Oxygen or nitrogen atoms or both are generally present in ether, ester, urethane, amide, and urea groups. Ethylenically unsaturated compounds may have a molecular weight of less than about 4,000 and may be esters made from the reac-

tion of compounds containing aliphatic monohydroxy groups or aliphatic polyhydroxy groups and unsaturated carboxylic acids, such as acrylic acid, methacrylic acid, itaconic acid, crotonic acid, isocrotonic acid, maleic acid, and the like. Representative examples of acrylate resins include methyl

methacrylate, ethyl methacrylate styrene, divinylbenzene, vinyl toluene, ethylene glycol diacrylate, ethylene glycol methacrylate, hexanediol diacrylate, triethylene glycol dia-

crylate, trimethylolpropane triacrylate, glycerol triacrylate, pentaerythritol triacrylate, pentaerythritol methacrylate, pentaerythritol tetraacrylate and pentaerythritol tetraacrylate. Other ethylenically unsaturated resins include monoallyl, polyallyl, and polymethallyl esters and amides of carboxylic acids, such as diallyl phthalate, diallyl adipate, and N,N-diallyl adipamide. Still other nitrogen containing compounds

include tris(2-acryloyloxyethyl)isocyanurate, 1,3,5-tri(2-methacryloyloxyethyl)-triazine, acrylamide, methylacrylamide, N-methylacrylamide, N,N-dimethylacrylamide, N-vinylpyrrolidone, and N-vinylpiperidone.

The aminoplast resins have at least one pendant  $\alpha,\beta$ -unsaturated carbonyl group per molecule or oligomer. These unsaturated carbonyl groups can be acrylate, methacrylate, or acrylamide type groups. Examples of such materials include

N-(hydroxymethyl) acrylamide, N,N'-oxydimethylenebisacrylamide, ortho- and para-acrylamidomethylated phenol, acrylamidomethylated phenolic novolac, and combinations thereof. These materials are further described in U.S. Pat. Nos. 4,903,440 and 5,236,472 both incorporated herein by reference.

Isocyanurate derivatives having at least one pendant acrylate group and isocyanate derivatives having at least one pendant acrylate group are further described in U.S. Pat. No. 4,652,274 incorporated herein after by reference. The isocyanurate material may be a triacrylate of tris(hydroxy ethyl) isocyanurate.

Epoxy resins have an oxirane and are polymerized by the ring opening. Such epoxide resins include monomeric epoxy resins and oligomeric epoxy resins. Examples of some useful epoxy resins include 2,2-bis[4-(2,3-epoxypropoxy)-phenyl propane](diglycidyl ether of Bisphenol) and commercially available materials under the trade designations "Epon 828", "Epon 1004", and "Epon 1001F" available from Shell Chemical Co., Houston, Tex., "DER-331", "DER-332", and "DER-334" available from Dow Chemical Co., Freeport, Tex. Other suitable epoxy resins include glycidyl ethers of phenol formaldehyde novolac (e.g., "DEN-431" and "DEN-428" available from Dow Chemical Co.).

Epoxy resins useful in the invention can polymerize via a cationic mechanism with the addition of an appropriate cationic curing agent. Cationic curing agents generate an acid source to initiate the polymerization of an epoxy resin. These cationic curing agents can include a salt having an onium cation and a halogen containing a complex anion of a metal or metalloid. Other cationic curing agents include a salt having an organometallic complex cation and a halogen containing complex anion of a metal or metalloid which are further described in U.S. Pat. No. 4,751,138 incorporated herein after by reference (column 6, line 65 to column 9, line 45). Another example is an organometallic salt and an onium salt is described in U.S. Pat. No. 4,985,340 (column 4, line 65 to column 14, line 50); and European Patent Application Nos. 306,161 and 306,162, both published Mar. 8, 1989, all incorporated by reference. Still other cationic curing agents include an ionic salt of an organometallic complex in which the metal is selected from the elements of Periodic Group IVB, VB, VIB, VIIIB and VIIIB which is described in European Patent Application No. 109,581, published Nov. 21, 1983, incorporated by reference.

Regarding free radical curable resins, in some embodiments the polymeric precursor solution may further comprise a free radical curing agent. However in the case of an electron beam energy source, the curing agent is not always required because the electron beam itself generates free radicals. Examples of free radical thermal initiators include peroxides, e.g., benzoyl peroxide, azo compounds, benzophenones, and quinones. For either ultraviolet or visible light energy source, this curing agent is sometimes referred to as a photoinitiator. Examples of initiators, that when exposed to ultraviolet light generate a free radical source, include but are not limited to those selected from organic peroxides, azo compounds, quinones, benzophenones, nitroso compounds, acryl halides, hydrozones, mercapto compounds, pyrlyium compounds, triacrylimidazoles, bisimidazoles, chloroalkytriazines, benzoin ethers, benzil ketals, thioxanthones, and acetophenone derivatives, and mixtures thereof. Examples of initiators that when exposed to visible radiation generate a free radical source can be found in U.S. Pat. No. 4,735,632, incorporated herein by reference. The initiator for use with visible light

may be that known under the trade designation "Irgacure 369" commercially available from Ciba Specialty Chemicals, Tarrytown, N.Y.

#### Other Optional Matrix Additives

Besides the materials described above, polymeric matrices useful in the invention may include effective amounts of other materials or components depending upon the end properties desired. For example, the polymeric matrix may include a shape stabilizer, i.e., a thermoplastic polymer with a melting point higher than that described above for the thermoplastic material. Suitable shape stabilizers include, but are not limited to, poly(phenylene sulfide), polyimides, and polyaramids. An example of a preferred shape stabilizer is polyphenylene oxide nylon blend commercially available from GE Plastics, Pittsfield, Mass., under the trade designation "Noryl GTX 910." If a phenolic-based coating is employed, however, the polyphenylene oxide nylon blend may not be preferred because of possible nonuniform interaction between the phenolic resin coating and the nylon, resulting in reversal of the shape-stabilizing effect. This nonuniform interaction results from a difficulty in obtaining uniform blends of the polyphenylene oxide and the nylon.

#### Oilfield Elements, Assemblies, and Wellbores

An "oilfield assembly", as used herein, is the complete set or suite of oilfield elements that may be used in a particular job. All oilfield elements in an oilfield assembly may or may not be interconnected, and some may be interchangeable.

An "oilfield element" includes, but is not limited to one or more items or assemblies selected from tubing, blow out preventers, sucker rods, O-rings, T-rings, jointed pipe, electric submersible pumps, packers, centralizers, hangers, plugs, plug catchers, check valves, universal valves, spotting valves, differential valves, circulation valves, equalizing valves, safety valves, fluid flow control valves, connectors, disconnect tools, downhole filters, motorheads, retrieval and fishing tools, bottom hole assemblies, seal assemblies, snap latch assemblies, anchor latch assemblies, shear-type anchor latch assemblies, no-go locators, and the like.

A "packer" is a device that can be run into a wellbore with a smaller initial outside diameter that then expands externally to seal the wellbore. Packers employ flexible, elastomeric seal elements that expand. The two most common forms are the production or test packer and the inflatable packer. The expansion of the former may be accomplished by squeezing the elastomeric elements (somewhat doughnut shaped) between two plates or between two conical frusta pointed inward, forcing the elastomeric elements' sides to bulge outward. The expansion of the latter may be accomplished by pumping a fluid into a bladder, in much the same fashion as a balloon, but having more robust construction. Production or test packers may be set in cased holes and inflatable packers may be used in open or cased holes. They may be run down into the well on wireline, pipe or coiled tubing. Some packers are designed to be removable, while others are permanent. Permanent packers are constructed of materials that are easy to drill or mill out. A packer may be used during completion to isolate the annulus from the production conduit, enabling controlled production, injection or treatment. A typical packer assembly incorporates a means of securing the packer against the casing or liner wall, such as a slip arrangement, and a means of creating a reliable hydraulic seal to isolate the annulus, typically by means of an expandable elastomeric element. Packers are classified by application, setting method and possible retrievability. Inflatable packers are capable of relatively large expansion ratios, an important factor in through-tubing work where the tubing size or completion

components can impose a significant size restriction on devices designed to set in the casing or liner below the tubing. Seal elements may either be bonded-type, using nitrile rubber seal elements, or chevron-type, available with seal elements comprising one or more proprietary elastomers such as those known under the trade designations Viton®, as mentioned above, available from DuPont Dow Elastomers LLC, and Aflas®, as mentioned above, available from Asahi Glass Co., Ltd. Bonded-type and chevron-type seal elements may both comprise one or more thermoplastic polymers, such as the polytetrafluoroethylene known under the trade designation Teflon®, available from E.I. DuPont de Nemours & Company; the polyphenylene sulfide thermoplastics known under the trade designation Ryton® and polyphenylene sulfide-based alloys known under the trade designation Xtel®, both available from Chevron Phillips Chemical Company LP. Both bond-type and chevron-type seal elements are available from Schlumberger.

A “wellbore” may be any type of well, including, but not limited to, a producing well, a non-producing well, an injection well, a fluid disposal well, an experimental well, an exploratory well, and the like. Wellbores may be vertical, horizontal, deviated some angle between vertical and horizontal, and combinations thereof, for example a vertical well with a non-vertical component.

FIGS. 1-6 illustrate several oilfield assemblies having one or more oilfield elements that may benefit from use of a nanoflake and/or nanoplatelet polymer composite. When an oilfield element is referred to by numeral, if that oilfield element may comprise a coated polymeric matrix it will be indicated with an asterisk (\*). It will be understood that not all of the described oilfield assemblies that may comprise a polymeric matrix need be the same in composition; indeed, not all of the possible oilfield elements need have a polymeric matrix. In some embodiments, perhaps only the protector bag of a submersible pump, for example, may be comprised of a nanoflake and/or nanoplatelet polymeric matrix. Further, when an oilfield element is mentioned as being comprised of a nanoflake and/or nanoplatelet polymeric matrix, the polymeric matrix may itself be a component of a larger structure, for example coated onto or placed adjacent another material, for example a metallic component.

FIG. 1 illustrates a first oilfield assembly 10 designed for deployment in a well 18 within a geological formation 20 containing desirable production fluids, such as petroleum. In a typical application, a wellbore 22 is drilled and lined with a wellbore casing 24. Wellbore casing 24 typically has a plurality of openings 26, for example perforations, through which production fluids may flow into wellbore 22.

Oilfield assembly 10 is deployed in wellbore 22 by a deployment system 28 that may have a variety of forms and configurations. For example, deployment system 28 may comprise tubing 30 connected to pump 12\* by a connector 32\*. Power is provided to a submersible motor 14\* via a power cable 34\*. Motor 14\*, in turn, powers centrifugal pump 12\*, which draws production fluid in through a pump intake 36\* and pumps the production fluid to the surface via tubing 30.

It should be noted that the illustrated oilfield assembly 10 is merely an exemplary embodiment. Other oilfield elements may be added to the oilfield assembly, and other deployment systems may be implemented. Additionally, the production fluids may be pumped to the surface through tubing 30 or through the annulus formed between deployment system 28 and wellbore casing 24. In any of these configurations of oilfield assembly 10, it may be desirable to be able to use two or more centrifugal pump stages having different operating

characteristics. Tubing 30 may be replaced by jointed pipe, which may include flanges and in that case flange gaskets\*.

In certain embodiments, oilfield assembly 10 may have one or more sections of motor protector 16\* disposed about motor 14\*. A schematic cross-sectional view of an exemplary embodiment of oilfield assembly 10 is provided in FIG. 2. As illustrated, oilfield assembly 10 comprises pump 12\*, motor 14\*, and various motor protection components disposed in a housing 38. Pump 12\* is rotatably coupled to motor 14\* via 10 a shaft 40, which extends lengthwise through the housing 38 (for example, one or more housing sections coupled together). Oilfield assembly 10 and shaft 40 may have multiple sections, which can be intercoupled via couplings and flanges. For example, shaft 40 has couplings 42\* and 44\* and 15 an intermediate shaft section 46 disposed between pump 12\* and motor 14\*.

A variety of seals, filters, absorbent assemblies and other protection elements also may be disposed in housing 38 to 20 protect motor 14\*. A thrust bearing 48\* is disposed about shaft 40 to accommodate and support the thrust load from pump 12\*. A plurality of shaft seals, such as shaft seals 50\* and 52\*, are also disposed about shaft 40 between pump 12\* and motor 14\* to isolate a motor fluid 54 in motor 14\* from 25 external fluids, such as well fluids and particulates. Shaft seals 50\* and 52\* also may include stationary and rotational components, which may be disposed about shaft 40 in a variety of 30 configurations. Oilfield assembly 10 also may include a plurality of moisture absorbent assemblies, such as moisture absorbent assemblies 56, 58, and 60, disposed throughout 35 housing 38 between pump 12\* and motor 14\*. These moisture absorbent assemblies 56-60 absorb and isolate undesirable fluids (for example, water, H<sub>2</sub>S, and the like) that have entered or may enter housing 38 through shaft seals 50\* and 52\* or through other locations. For example, moisture absorbent assemblies 56 and 58 may be disposed about shaft 40 at 40 a location between pump 12\* and motor 14\*, while moisture absorbent assembly 60 may be disposed on an opposite side of motor 14\* adjacent a protector bag 64\*. In addition, the actual protector section above the motor may include a hard bearing head with shedder.

As illustrated in FIG. 2, motor fluid 54 is in fluid communication with an interior 66\* of protector bag 64\*, while well fluid 68 is in fluid communication with an exterior 70\* of protector bag 64\*. Accordingly, protector bag 64\* seals motor fluid 54 from well fluid 68, while positively pressurizing motor fluid 54 relative to the well fluid 68 (e.g., a 50 psi pressure differential). The ability of elastomeric protector bag 64\* to stretch and retract ensures that motor fluid 54 maintains a higher pressure than that of well fluid 68. A separate spring assembly or biasing structure also may be incorporated in protector bag 64\* to add to the resistance, which ensures that motor fluid 54 maintains a higher pressure than that of well fluid 68.

Protector bag 64\* may embody a variety of structural features, geometries and materials as known in the art to utilize the pressure of well fluid 68 in combination with the stretch and retraction properties of protector bag 64\* to positively pressurize motor fluid 54. Initially, motor fluid 54 is injected into motor 14\* and protector bag 64\* is pressurized until a 55 desired positive pressure is obtained within motor 14\*. For example, oilfield assembly 10 may set an initial pressure, such as 25-100 psi, prior to submerging into the well. An exterior chamber 70 adjacent protector bag 64\* also may be filled with fluid prior to submerging the system into the well. Well fluid 68 enters housing 38 through ports 72 and mixes 60 with this fluid in exterior chamber 70 as oilfield assembly 10 is submersed into the well. Protector bag 64\* also may have 65

various protection elements to extend its life and to ensure continuous protection of motor 14\*. For example, a filter 74 may be disposed between ports 72 and exterior chamber 70 of protector bag 64\* to filter out undesirable fluid elements and particulates in well fluid 68 prior to fluid communication with exterior chamber 70. A filter 76 also may be provided adjacent interior 66\* of protector bag 64\* to filter out motor shavings and particulates. As illustrated, filter 76 is positioned adjacent moisture absorbent assembly 60 between motor cavity 62 and interior 66\* of protector bag 64\*. Accordingly, filter 76 prevents solids from entering or otherwise interfering with protector bag 64\*, thereby ensuring that protector bag 64\* is able to expand and contract along with volume variations in the fluids.

A plurality of expansion and contraction stops also may be disposed about protector bag 64\* to prevent over and under extension and to prolong the life of protector bag 64\*. For example, a contraction stop 78\* may be disposed within interior 66\* of protector bag 64\* to contact an end section 80\* and limit contraction of protector bag 64\*. An expansion stop 82\* also may be provided at exterior 70\* of protector bag 64\* to contact end section 80\* and limit expansion of the protector bag. These contraction and expansion stops 78\* and 82\* may have various configurations depending on the elastomer utilized for protector bag 64\* and also depending on the pressures of motor fluid 54 and well fluid 68. A housing 84\* also may be disposed about exterior 70\* to guide protector bag 64\* during contraction and expansion and to provide overall protection about exterior 70\*.

As oilfield assembly 10 is submersed and activated in the downhole environment, the internal pressure of motor fluid 54 may rise and/or fall due to temperature changes, such as those provided by the activation and deactivation of motor 14\*. A valve 86\* may be provided to release motor fluid 54 when the pressurization exceeds a maximum pressure threshold. In addition, another valve may be provided to input additional motor fluid when the pressurization falls below a minimum pressure threshold. Accordingly, the valves maintain the desired pressurization and undesirable fluid elements are repelled from motor cavity 62 at the shaft seals 50\* and 52\*. Oilfield assembly 10 also may have a wiring assembly 87\* extending through housing 38 to a component adjacent protector bag 64\*. For example, a variety of monitoring components may be disposed below protector bag 64\* to improve the overall operation of oilfield assembly 10. Exemplary monitoring components comprise temperature gauges, pressure gauges, and various other instruments, as should be appreciated by those skilled in the art.

FIG. 3 is a schematic perspective view, partially in cross-section, and not necessarily to scale, of another oilfield assembly 100 in accordance with the invention, in this case a packer. Although oilfield assembly 100 comprises in many instances more than one oilfield element, such as production tubing 104 and packer elements 108, oilfield assembly 100 is often referred to as a packer, and therefore this oilfield assembly may be considered an oilfield element which is part of a larger oilfield assembly, such as oilfield assembly 10 of FIGS. 1 and 2. A production liner or casing 102 is shown, partially broken away to reveal production tubing 104, hold-down slips 106, set-down slips 110, and a plurality of packer elements 108\* which, when expanded, produce a hydraulic seal between a lower annulus 109 and an upper annulus 111.

FIGS. 4A and 4B illustrate how two actuation arrangements may be used to directly override two flapper-style check valves, allowing uphole flow in a flow reversing oilfield assembly. The flow reversing oilfield assembly 150 illustrated schematically in FIG. 4A may include a motor 152\*, motor

shaft 153, and movable valve gate 156 positioned in a secondary channel 154, which moves dual flapper actuators 157 and 159, each having a notch 158 and 160, respectively. Movement up of shaft 153, gate 156, actuators 157 and 159, and notches 158 and 160 mechanically opens flappers 162 and 164, allowing reverse flow up tubing primary flow channel 151. O-ring seals 166\* and 168\* isolate production fluid from motor fluid 172. The flow reversing oilfield assembly 180 illustrated in FIG. 4B uses dual solenoids 184 and 182 to charge a hydraulic system and release the pressure. When the hydraulic system is charged, the hydraulic pressure in conduits 185, 185a, and 185b shift pistons 191 and 192, mechanically opening flappers 162 and 164, while high pressure below flapper 165 opens it, allowing reverse flow up tubing primary channel 151. When it is desired to stop reverse flow, or power or communication is lost, solenoid 184 is activated, releasing hydraulic pressure in conduits 185, 185a, and 185b, allowing flappers 162 and 164 to close in safe position. Note that an oil compensation system 194 may be used to protect and lubricate the motor, gears, and other mechanical parts, such as ball 193\* and spring 195\* of a check valve. Alternatively, these parts may be comprised of coated polymeric substrates in accordance with the invention. Various O-ring seals, such as seals 196\* and 197\* may be comprised of coated polymeric substrate, such as coated elastomers.

FIGS. 5A and 5B illustrate two oilfield assemblies 200 and 250 known as bottom hole assemblies, or BHAs. Bottom hole assemblies have many wellbore elements that may benefit from use of nanoflake and/or nanoplatelet polymeric composites in accordance with the teachings of the invention. The lower portion of the drillstring, consisting of (from the bottom up in a vertical well) the bit, bit sub, a mud motor (in certain cases), stabilizers, drill collars, heavy-weight drillpipe, jarring devices ("jars") and crossovers for various threadforms. The bottomhole assembly must provide force for the bit to break the rock (weight on bit), survive a hostile mechanical environment and provide the driller with directional control of the well. Oftentimes the assembly includes a mud motor, directional drilling and measuring equipment, measurements-while-drilling (MWD) tools, logging-while-drilling (LWD) tools and other specialized devices. A simple BHA may comprise a bit, various crossovers, and drill collars, however they may include many other wellbore elements leading to a relatively complex wellbore assembly.

Each oilfield assembly 200 and 250 may comprise tubing 202, a connector 204\*, a check valve assembly 206\*, and a pressure disconnect 208\*. Oilfield assembly 200 is a straight hole BHA, and includes drill collars 210, a mud pump 216\*, and a drill bit 220. Oilfield assembly 250 is a BHA for buildup and horizontal bore holes, and includes an orienting tool 212\*, an MWD section in a non-magnetic drill collar 214, mud pump 216\*, and drill bit 220, as well as an adjustable bent housing 218\*.

FIGS. 6A and 6B are schematic cross-sectional views of a flow control valve that may be utilized to control the flow of petroleum production or well fluids out of specific zones in a well or reservoir, or injection of fluid into specific zones, the valve utilizing nanoflake and/or nanoplatelet polymeric matrix components in accordance with the invention. These flow control valves may be operated by forces produced and controlled hydraulically, electrically or by a hybrid combination of appropriate electric and hydraulic components.

FIGS. 6A and 6B illustrate one embodiment of a hydraulically actuated valve. An inner tubular member 300 is contained within an actuator housing 301. A sliding sleeve 302 is equipped with sliding seals 303\*, 304\* and 305\*, thereby defining a confined volume chamber 306 and a controlled

volume chamber 307. If confined volume chamber 306 is pre-charged with a relatively inert gas such as nitrogen at sufficiently high pressure compared to the pressure in controlled volume chamber 307, then sliding sleeve 302 will be forced to the right, thereby closing fluid flow through an opening 309 in inner tubing 300 and an opening 311 in sliding sleeve 302. A seal 310 prevents the flow of fluid between tubular member 300 and sliding sleeve 302. If hydraulic oil is introduced into a tube 308 at a sufficiently high pressure then the force produced within controlled volume chamber 307 will be sufficient to overcome the force due to the pressurized gas in confined volume chamber 306 thereby resulting in sliding sleeve 302 moving to the left as illustrated in FIG. 6B. In FIG. 6B the movement of sliding sleeve 302 is sufficient to position opening 309 of inner tubular member 300 directly in-line with opening 311 in sliding sleeve 302. In this controlled configuration production fluid 312 can enter into the tubular member and thereby be unimpeded to flow into the tubing and up to the surface, assuming there is a fluid flow path and that the pressure is sufficient to lift the fluid to surface.

Sliding seals 303, 304, and 305 may be comprised of at least one of: O-rings, T-seals, chevron seals, metal spring energized seals, or combination of these to make a seal stack.

In application, sealing elements tend to adhere to one or both interface metal surfaces of the valve or sealed assembly. This can result in fluid or gas leaking through static or dynamic valve seals. In static, or non-moving seals, destructive mechanical stresses may also result from the difference in coefficient of thermal expansion of the mating parts made of differing materials, for example elastomers, polymers, metals or ceramics, or composites of these materials. Although the sealing element may change very little in size between hot and cold conditions, its expansion or contraction is relatively insignificant compared to the adjacent metal sealing elements or the valve, and since sealing elements are mechanically stressed with every thermal cycle, the sealing element eventually fractures thereby allowing fluid or gas to escape.

The polymer coating discussed herein, if used, may significantly improve the performance and lifetime of static seals and dynamic (or sliding sleeve) seals in the aforementioned fluid flow control valves by virtue of the coating's lubricant and wear resistance characteristics and its relative impermeability to gases and fluids. For example a 2  $\mu\text{m}$  coating imparts dry lubricant and wear resistance characteristics to the surface of the sliding seals. The lubricity of coating such as Parylene allows the sealing element to slide across the valve surfaces rather than sticking, thereby accommodating expansion and contraction differences that can fracture the seal. Since the sealing elements are not damaged in use, they can serve their intended sealing function and leaks are eliminated during a long functional life.

As may be seen by the exemplary embodiments illustrated in FIGS. 1-6 there are many possible uses of nanoflake and/or nanoplatelet polymeric matrices formed into oilfield elements and assemblies. Alternatives are numerous. For example, certain electrical submersible pumps, which are modified versions of a pumping system known under the trade designation Axia™, available from Schlumberger Technology Corporation, may feature a simplified two-component pump-motor configuration. Pumps of this nature generally have two stages inside a housing, and a combined motor and protector bag, which may be comprised of a coated polymeric substrate in accordance with the invention. This type of pump may be built with integral intakes and discharge heads. Fewer mechanical connections may contribute to faster installation and higher reliability of this embodiment. The combined

motor and protector assembly is known under the trade designation ProMotor™, and may be pre-filled in a controlled environment. The pump may include integral instrumentation that measures downhole temperatures and pressures.

Other alternative electrical submersible pump configurations that may benefit from components comprised of nanoflake and/or nanoplatelet polymer matrices include an ESP deployed on cable, an ESP deployed on coiled tubing with power cable strapped to the outside of the coiled tubing (the tubing acts as the producing medium), and more recently a system known under the trade designation REDACoil™, having a power cable deployed internally in coiled tubing. Certain pumps may have "on top" motors that drive separate pump stages, all pump stages enclosed in a housing. A separate protector bag is provided, as well as an optional pressure/temperature gauge. Also provided in this embodiment may be a sub-surface safety valve (SSSV) and a chemical injection mandrel. A lower connector may be employed, which may be hydraulically releasable with the power cable, and may include a control line and instrument wire feedthrough. A control line set packer completes this embodiment. The technology of bottom intake ESPs (with motor on the top) has been established over a period of years. It is important to securely install pump stages, motors, and protector within coiled tubing, enabling quicker installation and retrieval times plus cable protection and the opportunity to strip in and out of a live well. This may be accomplished using a deployment cable, which may be a cable known under the trade designation REDACoil™, including a power cable and flat pack with instrument wire and one or more, typically three hydraulic control lines, one each for operating the lower connector release, SSSV, and packer setting/chemical injection. Any one or more of the deployment cable, power cable, SSSV, control line set packer, chemical injection mandrel, and the like may comprise a polymeric matrix comprising nanoflakes and/or nanoplatelets, either in their O-ring seals or gaskets, as jackets for cables, as protector bags, and the like.

Oilfield assemblies of the invention may include many optional items. One optional feature may be one or more sensors located at the protector bag to detect the presence of hydrocarbons (or other chemicals of interest) in the internal motor lubricant fluid. The chemical indicator may communicate its signal to the surface over a fiber optic line, wire line, wireless transmission, and the like. When a certain chemical is detected that would present a safety hazard or possibly damage a motor if allowed to reach the motor, the pump may be shut down long before the chemical creates a problem.

In summary, generally, this invention pertains primarily to oilfield elements and assemblies comprising a polymeric matrix comprising nanoflakes and/or nanoplatelets, and optionally a coating, which may be a conformal protective coating deposited onto the polymeric matrix, where the polymeric matrix may be a thermoplastic, thermoset, elastomeric, or composite material. Methods of using the inventive oilfield elements and assemblies are also described.

Although only a few exemplary embodiments of this invention have been described in detail above, those skilled in the art will readily appreciate that many modifications are possible in the exemplary embodiments without materially departing from the novel teachings and advantages of this invention. Accordingly, all such modifications are intended to be included within the scope of this invention as defined in the following claims. In the claims, no clauses are intended to be in the means-plus-function format allowed by 35 U.S.C. § 112, paragraph 6 unless "means for" is explicitly recited together with an associated function. "Means for" clauses are

## 25

intended to cover the structures described herein as performing the recited function and not only structural equivalents, but also equivalent structures.

What is claimed is:

## 1. An apparatus comprising:

- (a) a polymeric matrix formed into an oilfield element; and
- (b) a plurality of expanded graphitic nanoflakes and/or nanoplatelets having an expansion ratio ranging from about 40:1 to about 300:1 dispersed in the polymeric matrix, wherein the expanded graphitic nanoflakes and/or nanoplatelets are selected from the group consisting of expanded graphite, exfoliated graphite, and compositions based on boron and nitrogen, and mixtures and combinations thereof.

2. The apparatus of claim 1 wherein the expanded graphitic nanoflakes and/or nanoplatelets have aspect ratio exceeding 100.

3. The apparatus of claim 1 wherein the polymeric matrix comprises expanded and/or exfoliated graphitic nano flakes and/or nanoplatelets with aspect ratio less than 200.

4. The apparatus of claim 2 wherein the polymeric matrix comprises expanded and/or exfoliated graphitic nanoflakes and/or nanoplatelets with aspect ratio less than 200.

5. The apparatus of claim 1 wherein the polymeric matrix includes both expanded graphitic platelets with aspect ratio less than 200 and exceeding 200.

6. The apparatus of claim 1 wherein the expanded graphitic nanoflakes and/or nanoplatelets assume heterogeneous forms.

7. The apparatus of claim 1 wherein the polymeric matrix comprises one or more polymers selected from the group consisting of natural and synthetic polymers.

8. The apparatus of claim 1 wherein the oilfield element is selected from the group consisting of tubing, jointed pipe, sucker rods, electric submersible pumps, submersible pump motor protector bags, packers, packer elements, blow out preventers, blow out preventer elements, O-rings, T-rings, centralizers, hangers, plugs, plug catchers, check valves, universal valves, spotting valves, differential valves, circulation valves, equalizing valves, safety valves, fluid flow control valves, sliding seals, connectors, disconnect tools, downhole filters, motorheads, retrieval and fishing tools, bottom hole assemblies, seal assemblies, snap latch assemblies, anchor latch assemblies, shear-type anchor latch assemblies, no-go locators, sensor protectors, gaskets, pump shaft seals, tube seals, valve seals, seals and insulators used in electrical components, seals used in fiber optic connections, pressure sealing elements for fluids and combinations thereof.

## 9. An apparatus comprising:

- (a) a polymeric matrix formed into an oilfield element; and
- (b) a plurality of expanded graphitic nanoflakes and/or nanoplatelets having an expansion ratio ranging from about 40:1 to about 300:1 dispersed in the polymeric matrix, wherein the nanoflakes and/or nanoplatelets have thickness of about 0.3 nm to about 100 nm, and lateral size of about 5 nm to about 500 nm.

## 10. An apparatus comprising:

- (a) a polymeric matrix formed into an oilfield element; and
- (b) a plurality of expanded graphitic nanoflakes and/or nanoplatelets having an expansion ratio ranging from about 40:1 to about 300:1 dispersed in the polymeric matrix, wherein some or all of the expanded graphitic nanoflakes, or portions of each nanoflake, have 3-dimensional shapes selected from the group consisting of substantially flat and other than flat.

11. The apparatus of claim 10 wherein the 3-dimensional shape other than flat is selected from the group consisting of

## 26

saddles, half-saddles, quarter-saddles, half-spheres, quarter spheres, cones, half-cones, bells, half-bells, horns, and quarter-horns.

## 12. An apparatus comprising:

- (a) a polymeric matrix formed into an oilfield element; and
- (b) a plurality of expanded graphitic nanoflakes and/or nanoplatelets having an expansion ratio ranging from about 40:1 to about 300:1 dispersed in the polymeric matrix, wherein at least a portion of the expanded graphitic nanoflakes and/or platelets are surface modified.

## 13. An oilfield element comprising:

- (a) a polymeric matrix formed into at least a portion of the oilfield element; and
- (b) a plurality of expanded graphitic nanoflakes and/or nanoplatelets having an expansion ratio ranging from about 40:1 to about 300:1 dispersed in the polymeric matrix, wherein the expanded graphitic nanoflakes and/or nanoplatelets are selected from the group consisting of expanded graphite, exfoliated graphite, and compositions based on boron and nitrogen, and mixtures and combinations thereof.

14. The oilfield element of claim 13 wherein the polymeric matrix comprises one or more polymers selected from the group consisting of natural and synthetic polymers.

15. The oilfield element of claim 13 selected from the group consisting of tubing, jointed pipe, sucker rods, electric submersible pumps, submersible pump motor protector bags, packers, packer elements, blow out preventers, blow out preventer elements, O-rings, T-rings, centralizers, hangers, plugs, plug catchers, check valves, universal valves, spotting valves, differential valves, circulation valves, equalizing valves, safety valves, fluid flow control valves, sliding seals, connectors, disconnect tools, downhole filters, motorheads, retrieval and fishing tools, bottom hole assemblies, seal assemblies, snap latch assemblies, anchor latch assemblies, shear-type anchor latch assemblies, no-go locators, sensor protectors, gaskets, pump shaft seals, tube seals, valve seals, seals and insulators used in electrical components, seals used in fiber optic connections, pressure sealing elements for fluids and combinations thereof.

16. An oilfield assembly for exploring for, drilling for, or producing hydrocarbons, comprising:

- (a) one or more oilfield elements selected from the group consisting of tubing, jointed pipe, sucker rods, electric submersible pumps, submersible pump motor protector bags, packers, packer elements, blow out preventers, blow out preventer elements, O-rings, T-rings, centralizers, hangers, plugs, plug catchers, check valves, universal valves, spotting valves, differential valves, circulation valves, equalizing valves, safety valves, fluid flow control valves, sliding seals, connectors, disconnect tools, downhole filters, motorheads, retrieval and fishing tools, bottom hole assemblies, seal assemblies, snap latch assemblies, anchor latch assemblies, shear-type anchor latch assemblies, no-go locators, sensor protectors, gaskets, pump shaft seals, tube seals, valve seals, seals and insulators used in electrical components, seals used in fiber optic connections, pressure sealing elements for fluids, and combinations thereof; and

- (b) one or more of the oilfield elements comprising a plurality of expanded graphitic nanoflakes and/or nanoplatelets having an expansion ratio ranging from about 40:1 to about 300:1 dispersed in a polymeric matrix, wherein the expanded graphitic nanoflakes and/or nanoplatelets are selected from the group consisting of

**27**

expanded graphite, exfoliated graphite, and compositions based on boron and nitrogen, and mixtures and combinations thereof.

**17. A method comprising:**

- (a) selecting one or more oilfield elements having a component comprising a plurality of expanded graphitic nanoflakes and/or nanoplatelets having an expansion ratio ranging from about 40:1 to about 300:1 dispersed in a polymeric matrix, wherein the expanded graphitic nanoflakes and/or nanoplatelets are selected from the group consisting of expanded graphite, exfoliated graphite, and compositions based on boron and nitrogen, and mixtures and combinations thereof; and
- (b) using the one or more oilfield element in an oilfield operation, thus exposing the oilfield element to an oilfield environment.

**18. The method of claim 17 wherein the oilfield element is selected from the group consisting of tubing, jointed pipe, sucker rods, electric submersible pumps, submersible pump motor protector bags, packers, packer elements, blow out preventers, blow out preventer elements, O-rings, T-rings,**

**28**

centralizers, hangers, plugs, plug catchers, check valves, universal valves, spotting valves, differential valves, circulation valves, equalizing valves, safety valves, fluid flow control valves, sliding seals, connectors, disconnect tools, downhole filters, motorheads, retrieval and fishing tools, bottom hole assemblies, seal assemblies, snap latch assemblies, anchor latch assemblies, shear-type anchor latch assemblies, no-go locators, sensor protectors, gaskets, pump shaft seals, tube seals, valve seals, seals and insulators used in electrical components, seals used in fiber optic connections, pressure sealing elements for fluids, and combinations thereof.

**19. A method comprising:**

- (a) selecting an electric submersible pump having a protector bag comprising a plurality of expanded graphitic nanoflakes and/or nanoplatelets dispersed in a polymeric matrix; and
- (b) using the electric submersible pump in an oilfield operation, thus exposing the protector bag to an oilfield environment.

\* \* \* \* \*